

## 1

3,658,704

**SYNERGISTIC GREASE STRUCTURE MODIFIERS**  
George G. Curtis, Westfield, N.J., assignor to Esso  
Research and Engineering Company  
No Drawing. Filed June 5, 1969, Ser. No. 830,846  
Int. Cl. C10m 5/14  
U.S. Cl. 252—42

8 Claims

### ABSTRACT OF THE DISCLOSURE

In a lubricating grease comprising a lubricating oil and a lithium soap of a C<sub>18</sub> hydroxy fatty acid, the improvement of using a synergistic combination of at least two different C<sub>2</sub>—C<sub>10</sub> aliphatic polyols for structural modification.

### BACKGROUND OF THE INVENTION

#### Field of the invention

This invention is directed to the improvement in lubricating grease compositions comprising a base lubricating oil and a lithium soap of a C<sub>18</sub> hydroxy fatty acid, of using a synergistic combination of at least two different C<sub>2</sub>—C<sub>10</sub> aliphatic polyols for structural modification.

More particularly it is directed to the use, in greases containing a lithium soap of a C<sub>18</sub> hydroxy fatty acid as a thickening agent, of a combination of at least two different aliphatic hydrocarbons, branched or straight chain, polyols consisting of carbon, hydrogen and oxygen and having 2 to 10 carbon atoms and 2 to 8 hydroxy groups per polyol in place of the individual hydroxyl substituted structural modifiers disclosed in the prior art.

#### Description of the prior art

U.S. Pat. 3,158,574 discloses that grease containing lithium hydroxy soaps as a gelling agent, having an improved structure, may be obtained by incorporating a glyceride in the constituents from which the acid constituents of the grease forming soap is derived. During manufacture the glyceride hydrolyzes resulting in a glycerol content of about 1.4 wt. percent based on the total composition which acts as a modifier. This patent further teaches that improved properties can also be obtained by the addition of an aliphatic polyhydroxy structure modifying agent. Among the aliphatic structure modifiers taught in said patent are glycols, polyglycols and partial esters of glycols in proportions of between 1% and 4% by wt. based on the total composition.

### SUMMARY OF THE INVENTION

It has now been discovered that the lubricating properties of hydroxy stearic acid soap greases such as those of said U.S. 3,158,574 can be even further improved by the addition of a combination of at least two different C<sub>2</sub>—C<sub>10</sub> aliphatic polyols as structural modifiers.

More specifically it has now been found that a combination of at least two of these modifying agents exert a synergistic improvement in structural stability and product yield over that obtainable with the use of a single modifier. In addition combinations of modifiers herein proposed generally produce a better grease having better shear and structural stability while requiring less modifier than the similar hydroxy soap grease systems employing a single modifier.

The combination of compounds contemplated for use in this invention are nonaromatic preferably saturated hydroxy materials of about 2 to 10 carbon atoms, preferably 3 to 6 carbon atoms and having 2 to 8, preferably 2 to 6 hydroxy groups. Such compounds include C<sub>5</sub>—C<sub>10</sub> alicyclic polyols, and C<sub>2</sub>—C<sub>10</sub> acyclic polyols.

## 2

Among the alicyclic compounds contemplated for use in this invention are 1,2-cyclopentanediol, 1,4-cyclohexanediol and 1,4-bis (hydroxymethyl) cyclohexane.

Preferred for use in this invention are combinations of C<sub>2</sub> to C<sub>10</sub> acyclic polyols. Especially preferred are the C<sub>3</sub> to C<sub>6</sub> acyclic polyols such as 1,2,3-propanetriol, 2-methyl, 2,4-pentanediol, 1,6-hexanediol, 1,2,6-hexanetriol, 1,2,3,4,5,6-hexanehexol, etc. Most preferred is a combination of sorbitol (which is 1,2,3,4,5,6-hexanehexol) and 1,6-hexanediol.

The weight percent of said combination of modifiers contemplated for use by this invention ranges from about 0.01 to 2% and, preferably, from 0.1 to 1% by weight based on the weight of the total grease composition.

While this invention contemplates the use of a combination of two or more modifiers, preferred is the use of a combination of two modifiers. The relative molar ratios of the two modifiers to each other range from about 1 to 4 to about 4 to 1, preferably 2 to 1 to about 1 to 2.

Most preferred is a combination of about equal molar amounts of modifiers.

The methods by which the greases employing the inventive synergistic modifiers are to be manufactured are known in the art. For example, see U.S. 3,158,574.

However, contrary to the teachings of U.S. 3,158,574 when using this combination of modifying agents it is no longer necessary to add them at a particular stage of grease manufacture and these modifiers can be added at any time before the grease begins to cool. However, the modifiers are especially effective when most of the cut-back oil is slowly added to the concentrated soap base while the temperature is maintained near the maximum manufacturing temperature.

The lubricating oil employed to produce lubricating grease compositions may be conventional grease-making mineral lubricating oils which are well-known in the art.

The hydroxy fatty acids used in forming the thickening agent for the grease is preferably a hydroxy stearic acid with 1 to 2 hydroxy groups such as 9-hydroxy stearic, 10-hydroxy stearic, 12-hydroxy stearic and 9,10-dihydroxy stearic acid, etc.

The total thickener content should range from about 3 to about 25 wt. percent and preferably 6—12 wt. percent of the total grease composition.

The nature of this invention will be further understood when reference is made to the following examples which include preferred embodiments which are not to be construed as a limitation of the invention.

50

### EXAMPLE 1

562 grams of 12-hydroxy stearic acid and 1500 grams of mineral lubricating oil having a V.I. of 85 and a viscosity of 700—775 SUS at 100° F. (hereinafter referred to as Oil A) were added to a laboratory grease kettle and were mixed at 160° F. Then 88.5 grams of lithium hydroxide (LiOH) were added and the heat was raised to 200° F. and held for one hour. The heat was then raised to 340° F. and 8 grams of sorbitol and 8 grams of 1,6-hexanediol were added. The temperature was then further raised to 380° F. and held for 1 hour. 1000 grams of the resulting mixture were then placed in a Hobart mixer and 2050 grams additional Oil A were added to cut back said mixture to a No. 1 grade grease.

65

### EXAMPLE 2

562 grams of 12-hydroxy stearic acid and 1500 grams of Oil A were added to a laboratory grease kettle and were mixed at 160° F. 88.5 grams of lithium hydroxide were then added and the heat was raised to 200° F. and held for 1 hour. The heat was then raised to 340° F. and

8 grams of sorbitol and 8 grams of 1,6-hexanediol pre-dissolved in 100 grams of Oil A were added. The temperature was then further raised to 380° F. and held for 1 hour. 1000 grams of the resulting mixture were then placed in a Hobart mixer and 2010 grams of additional Oil A were added to cut back said mixture to a No. 1 grade grease.

**Comparative Grease A—Effect of 1,6-hexanediol alone**

562 grams of 12-hydroxy stearic acid, 1500 grams of Oil A were blended together at 200° F. Then 88.5 grams of lithium hydroxide were added mixed at 250° F. for 1 hour. The temperature was then slowly increased to 350° F. and 16 grams of 1,6-hexanediol were added. The temperature was then increased to 390° F. and this temperature was kept constant for one hour. 1000 grams of the resulting mixture were then placed in the Hobart mixer and 2500 grams additional Oil A were added.

**EXAMPLE 3**

562 grams of 12-hydroxy stearic acid and 1500 grams of Oil A were added to a laboratory grease kettle and mixed at 150° F. 88.5 grams of lithium hydroxide were then added and the composition was mixed to 212° F. for one hour. The temperature was then slowly brought to 350° F. and 8 grams of sorbitol, 8 grams of 1,6-hexanediol and 200 grams of Oil A were added. The temperature was then further raised to 400° F. and 1800 grams additional Oil A and 6 grams phenyl alpha naphthylamine (an antioxidant) were added. The mixture was allowed to cool overnight. 220 grams of the resulting mixture were then combined with 480 grams of Oil A to produce the finished grease.

**Comparative Grease B—Effect of 1,6-hexanediol**

The procedure and materials of the Comparative Grease A were repeated except that 8 grams of 1,6-hexanediol were substituted for the 16 grams of 1,6-hexanediol used in Comparative Grease A.

**Comparative Grease C—Effect of sorbitol**

The procedure and materials of Comparative Grease A were repeated except that 8 grams of Sorbitol were substituted for the 16 grams of 1,6-hexanediol used in Comparative Grease A.

Table I, which follows, summarizes the composition and properties of the preceding greases. The percent soap and percent modifier in said table represent the approximate wt. percent found in the final grease composition.

sists of an outer steel cylinder 182 millimeters in length and 90 millimeters in inside diameter. This cylinder is permanently closed at one end while the other end is provided with a flange and a removable cover plate. An inner cylindrical roller 177 millimeters in length and 60 millimeters in outside diameter is filled with lead to give a weight of about 11 lbs. The outer cylinder has a wall thickness of 3 millimeters, and the same thickness of steel is soldered on each end of the inner cylinder so that no lead is exposed. The operation of this test equipment consists of placing a weighted amount of lubricating grease in the open cylinder, inserting the roller, closing the cylinder and rotating the cylinder at 160 r.p.m. for 4 hours. At the end of this period the test sample is removed and tested by means of a miniature penetrometer cone to determine any change in consistency. The figures in Table I represent the percentage of change.

Table I demonstrates the results of modifier synergism in greases. While the greases formed in Examples 1 and 2 and Comparative Grease A have about the same consistency, started off with the same relative proportions of starting materials and have about the same total modifier content, the synergistic combinations in Examples 1 and 2 exhibited far more stability than the single modifier in Comparative Grease A. The tests run on Comparative Greases B and C and the grease of Example 3 similarly demonstrate the synergism which occurs at even lower concentrations. Furthermore, the poor results shown by Comparative Greases B and C highlights the unobviousness of obtaining superior stability from a combination of these low modifier concentrations.

**EXAMPLE 4**

562 grams of 12-hydroxy stearic acid and 1500 grams of Oil A were added to a laboratory grease kettle and mixed at 150° F. 88.5 grams of lithium hydroxide were then added and the composition was mixed to 212° F. for one hour. The temperature was then slowly brought to 350° F. and 24 grams of sorbitol, 24 grams of 1,6-hexanediol and 200 grams of Oil A were added. The temperature was then further raised to 390° F. and 1800 grams additional Oil A and 6 grams phenyl alpha naphthylamine (an antioxidant) were added. 400 grams of the resulting mixture were then placed in a mixer together with 200 grams of additional Oil A to produce a finished grease.

**EXAMPLE 5**

562 grams of 12-hydroxy stearic acid and 1500 grams

TABLE I

|                                                               | Ex. 1 | Ex. 2 | Comparative<br>grease A | Ex. 3 | Comparative<br>grease B | Comparative<br>grease C |
|---------------------------------------------------------------|-------|-------|-------------------------|-------|-------------------------|-------------------------|
| Percent soap.....                                             | 9.0   | 8.8   | 11.3                    | 9.1   | 9.8                     | 7.2                     |
| Percent sorbitol.....                                         | 0.12  | 0.12  | -----                   | 0.06  | -----                   | 0.12                    |
| Percent 1,6-hexanediol.....                                   | 0.12  | 0.12  | 0.24                    | 0.06  | 0.12                    | -----                   |
| Dropping point, ° F.....                                      | 394   | 395   | -----                   | 381   | -----                   | -----                   |
| ASTM D-217 Penetration, mm./10 at<br>77° F.:                  |       |       |                         |       |                         |                         |
| Unworked.....                                                 | 319   | 321   | 298                     | ----- | 306                     | 304                     |
| Worked 60 strokes (60X).....                                  | 316   | 319   | 322                     | 311   | 306                     | 312                     |
| Worked 10,000 strokes.....                                    | 327   | 320   | -----                   | 310   | -----                   | -----                   |
| Worked 100,000 strokes (100MX).....                           | 319   | 307   | 367                     | 305   | 330                     | 336                     |
| Percent Δ (100MX-60X strokes).....                            | +1    | -3.8  | +14                     | -2    | +7.8                    | +7.8                    |
| ASTM D-1831-64 roll stability, per-<br>cent Δ in 4 hours..... | 10.3  | 9.1   | 40.0                    | 10.0  | 26.7                    | 20.8                    |

ASTM-D-217 can be used as a structural stability test to determine the ability of a grease to withstand prolonged use under severe working conditions. The working consists of placing the lubricating grease in a cylinder cup and operating a perforated plate for the number of strokes as indicated in Table I at 77° F. The percent of change of penetration at 60 strokes and at 100,000 strokes is then calculated and the lower the percent figure the more stable the grease.

The Roll Stability Test (ASTM-D-1831-64) is a test to measure stability toward shear. The equipment con-

65 of Oil A were added to a laboratory grease kettle and were mixed at 160° F. Then 88.5 grams of lithium hydroxide were added and the heat was raised to 200° F. and held for one hour. The heat was then raised to 340° 70 F. and 8 grams of sorbitol and 8 grams of glycerol were added. The temperature was then further raised to 380° F. and held for 1 hour. 1000 grams of the resulting mixture were then placed in a Hobart mixer and 1775 grams additional Oil A were added.

## 5 AMPLE 6

562 grams of 12-hydroxy stearic acid and 1500 grams of Oil A were added to a laboratory grease kettle and mixed at 150° F. 88.5 grams of lithium hydroxide were then added and the composition was mixed to 212° F. for one hour. The temperature was then slowly brought to 350° F. and 8 grams of sorbitol, 8 grams of 1,2,6-hexanetriol and 200 grams of Oil A were added. The temperature was then further raised to 390° F. and 1800 grams additional Oil A and 6 grams phenyl alpha naphthylamine (an antioxidant) were added.

635 grams of the resulting mixture were then placed in a mixer together with 165 grams of additional Oil A to produce a grease having an ASTM worked penetration after 60 strokes of 317 mm./10.

Table II illustrates the excellent properties of the greases formed in these examples using various concentrations and combinations of modifiers.

30 grams of water, were then added and the heat was raised to 200° F. and held for one hour. The temperature was then raised to 370° F. and two grams of glycerol and two grams of 1,2,6-hexanetriol were added and the temperature was raised to 40° F. The heat source was removed and the mixture was allowed to cool overnight quiescently. The product, which gelled after standing overnight, was milled in a three roll paint mill together with 375 additional grams of Oil B which were added to produce a No. 1 grade grease.

**EXAMPLE 9**

The procedure of Example 8 was repeated except two grams of sorbitol and two grams of 1,6-hexanediol were used instead of the two grams of glycerol and the two grams of 1,2,6-hexanetriol.

The products of these three examples were tested and Table III shows the results of these tests. Modifier percent and soap percent indicate the percent of soap and modifier present in the final grease composition.

TABLE III

|                                                | Example 7                          | Example 8                             | Example 9                          |
|------------------------------------------------|------------------------------------|---------------------------------------|------------------------------------|
| Modifier, percent                              | 1.0 sorbitol<br>1.0 1,6 hexanediol | 0.2 glycerol<br>0.2 1,2,6-hexanetriol | 0.2 sorbitol<br>0.2 1,6-hexanediol |
| Soap, percent                                  | 11                                 | 7                                     | 7                                  |
| ASTM Penetration, 77° F., mm./10:              |                                    |                                       |                                    |
| Unworked                                       | 295                                | 327                                   |                                    |
| Worked 60 strokes (60X)                        | 306                                | 334                                   | 316                                |
| Worked 10,000 strokes (10M)                    | 338                                | 360                                   | 307                                |
| Percent $\Delta$ (10MX-60X)                    | 10                                 | 8                                     | -3                                 |
| Static hardening, percent $\Delta$ in 28 days: |                                    |                                       |                                    |
| At 77° F.                                      | 47                                 | 28                                    | 19                                 |
| At 25° F.                                      | 49                                 | 38                                    | 27                                 |

TABLE II

|                                      | Ex. 4    | Ex. 5    | Ex. 6    |
|--------------------------------------|----------|----------|----------|
| Percent soap                         | 9.6      | 11.3     | 13.2     |
| Percent modifier                     | { 1 0.38 | { 1 0.13 | { 1 0.15 |
| Drop point, °F                       | { 2 0.38 | { 3 0.13 | { 4 0.15 |
| ASTM Penetrations, 77° F., mm./10:   |          |          |          |
| Worked 60 strokes (60X)              | 317      | 311      | 317      |
| Worked 10,000 strokes                |          | 320      |          |
| Worked 100,000 strokes (100MX)       | 315      | 309      | 324      |
| Percent Δ (100MX-60X strokes)        | -0.6     | -0.6     | +2.2     |
| Roll stability, percent Δ in 4 hours | 14.7     | 3.3      | 9.5      |

- <sup>1</sup> Sorbitol.
- <sup>2</sup> 1,6-hexanediol.
- <sup>3</sup> Glycerol.
- <sup>4</sup> 1,2,6-hexanetriol.

Example 4 illustrates the effectiveness of sorbitol and 1,6-hexanediol at higher concentrations and Examples 5 and 6 are illustrative of the effectiveness of other combinations of modifiers.

An additional batch of greases was prepared to demonstrate that greases with low soap content and good-to-excellent static hardening properties could be prepared by employing a combination of modifiers.

### EXAMPLE 7

75 grams of 12-hydroxy stearic acid and 600 grams of a mineral oil having a flash point of 388° F., a specific gravity of 22° API and a viscosity at 210° F. of 55 SUS (hereinafter referred to as Oil B) were blended together and heated to 160° F.; 10.5 grams of lithium hydroxide dissolved in 30 grams of water were then added. The mixture was heated to 200° F. and mixed for one hour. The temperature was then slowly increased to 360° F. Seven grams of sorbitol and seven grams of 1,6-hexane-diol were mixed together and added and the temperature was raised to 400° F. The heat source was then removed and the mixture was allowed to cool quiescently overnight. The product which gelled overnight was then milled.

### EXAMPLE 8

75 grams of 12-hydroxy stearic acid and 600 grams of Oil B were added to a Hobart mixer and heated to 160° F.; 10.5 grams of lithium hydroxide dissolved in

The static oven hardening test is a measure of the hardening of greases due to standing for periods of time. This is an important characteristic related to their performance in lubricating bearings. The test procedure consists essentially of initially working a grease 60 strokes with a penetration apparatus consisting of a modified cone, such cone producing penetrations about one-half the scale of penetration produced by the usual cones. The initially worked greases are then stored at room temperature and at a temperature of 250° F. After 1, 7 and 28 days, a penetration test using the modified cone is conducted on the stored unworked greases and the percentage of change in penetration is determined.

The present invention may be embodied in other specific forms without departing from the spirit or essential attributes thereof, and it is therefore desired that the present embodiments be considered in all respects as illustrative and not restrictive, reference being had to the appended claims rather than to the foregoing description to indicate the scope of the invention.

What is claimed is:

- 55 1. In a lubricating grease of the type comprising a major amount of lubricating oil and about 3 to about 25 wt. percent of a lithium soap of a C<sub>18</sub> hydroxy fatty acid as a thickening agent, the improvement comprising having in admixture with said oil about .01 to about 2 wt. percent of a synergistic stability-imparting combination of two different C<sub>2</sub>-C<sub>10</sub> aliphatic polyol modifier compounds in a relative molar ratio to each other ranging from about 4:1 to about 1:4.

60 2. The composition of claim 1 wherein said combination of two modifiers are C<sub>2</sub>-C<sub>10</sub> acyclic polyols.

65 3. The composition of claim 1 wherein the amount of hydroxyl substitution in each of the modifiers ranges from about two to about eight hydroxyl substitutions.

70 4. The composition of claim 1 wherein said combination of modifiers are C<sub>2</sub>-C<sub>6</sub> acyclic polyols.

5. The composition of claim 1 wherein the amount of hydroxyl substitution in each of the modifiers ranges from

hydroxyl substitution in each of the modifiers ranges from two to six hydroxyl substitutions.

6. The composition of claim 1 wherein the total amount of said combination of modifiers is between about 0.1 and about 1 wt. percent of the total composition.

7. The composition of claim 1 wherein said combination of modifiers is sorbitol and 1,6-hexanediol.

8. The composition of claim 1 wherein said combination of modifiers consists of two modifiers having a relative molar ratio to each other ranging from about 2:1 to about 1:2.

**References Cited**

**UNITED STATES PATENTS**

2,449,312 9/1948 Murray et al. ----- 252—42

|           |         |                        |          |
|-----------|---------|------------------------|----------|
| 2,606,874 | 8/1952  | Garner et al. -----    | 252—52   |
| 2,815,560 | 12/1957 | Buxton -----           | 252—56   |
| 3,158,574 | 11/1964 | Greenwood et al. ----- | 252—42   |
| 3,235,510 | 2/1966  | Collings et al. -----  | 252—33.4 |

<sup>5</sup> DANIEL E. WYMAN, Primary Examiner  
I. VAUGHN, Assistant Examiner

U.S. Cl. X.R.

10 252—52 R